

## UNITED STATES PATENT OFFICE

WILLY O. HERRMANN AND WOLFRAM HAEHNEL, OF MUNICH, GERMANY, ASSIGNEES  
TO CONSORTIUM FUR ELEKTROCHEMISCHE INDUSTRIE G. M. B. H., OF MUNICH,  
GERMANY, A CORPORATION OF GERMANY

## SHOE STIFFENER

No Drawing. Application filed May 31, 1929, Serial No. 367,610, and in Germany June 29, 1928.

This invention relates to shoe stiffeners for box toes and heel counters of shoes. These stiffeners are used to give the heel and toe portions of the shoe sufficient strength to retain its shape and are held in position by adhesion to the lining and the overlying leather of the shoe.

An object of this invention is to provide a shoe stiffener which can be economically made and safely handled by shoe factories. A further object is to provide an article that will permanently retain the necessary flexibility and will not contain substances which are injurious either to the foot or the leather of which the shoe is made. A still further object is to provide a material having great power of adhesion so that there is no danger of the lining or the leather of the shoe separating from the stiffening material.

Heretofore the most satisfactory stiffeners has been made by impregnating some suitable fabric, generally felt, with a cellulose ester solution such as celluloid. The use of such impregnating material has many disadvantages, one of the greatest objections being the high cost due to the fact that large volumes of solvent are necessary to incorporate a sufficient quantity of the cellulose ester in the fabric. It is obvious that to give the material sufficient strength, a considerable quantity of cellulose ester must be absorbed and it has been found impossible to keep high concentrations of ester in solution or to keep the viscosity sufficiently low to handle the impregnation from a practical point of view. As a result, several impregnations are necessary. Moreover, the stiffening material upon drying is too brittle and has a strong tendency to crack when the shoe is subjected to the ordinary strain encountered in wear. This latter objection has been overcome by the addition of plasticisers to the impregnating solution, the effect of which is to give the stiffening material a satisfactory initial flexibility, but this effect is not permanent, due to the fact that the plasticiser slowly volatilizes and leaves the material brittle. An added objection to this plasticiser is that it has an injurious effect on both the shoe leather and the foot.

It is apparent, therefore, that the addition of plasticisers is far from satisfactory.

A further disadvantage in the shoe stiffeners heretofore commonly used lies in the fact that the impregnating materials possess very inferior adhesive properties, giving no assurance that the stiffening material will permanently adhere to either the lining or the overlying leather of the shoe, and furthermore, a solvent of the cellulose ester must be brought in contact with the material to develop even this inferior adhesive property at all. This necessitates the use of the impregnated fabric while the impregnating solution is still wet, obviously an impractical procedure in a shoe factory, or the steaming of stiffener in some cellulose ester solvent just before use. As the solvent vapors suitable for the cellulose esters are extremely inflammable, this latter procedure is a source of constant danger and must necessarily be done in the immediate vicinity of the shoe factory in order to use the stiffener before the cellulose ester sets again.

We have found that by impregnating the stiffening material with a solution of poly vinyl acetate all of these disadvantages are overcome. The alcohol and benzene soluble modifications of poly vinyl acetate are particularly adapted for this use and have the added advantage of being readily soluble in relatively cheap solvents, alcohol and benzene. In contrast to the cellulose ester solutions, alcohol solutions of poly vinyl acetate can easily be made having a 60-70% poly vinyl acetate content and having relatively greater fluidity than the cellulose ester solutions of far lower solid content. A single impregnation of such a poly vinyl acetate solution gives the stiffener sufficient strength, whereas the cellulose ester solution has such a low solid content that several impregnations are necessary and as a result considerable quantities of valuable solvents are lost. The poly vinyl acetate has a remarkable power of adhesion far in excess of that of the cellulose esters and insures a permanent adhesion of the stiffener to the lining and leather of the shoe regardless of the strain put on the shoe by the wearer. An added

- advantage of our impregnating solution is that after the material has been impregnated and dried, the adhesive property of the poly vinyl acetate can be fully developed by merely heating the material to 60—80° C. at which temperature the leather is not injured and does not require any treatment with solvent vapors. Therefore the stiffening material can be impregnated and dried at some 10 remote place and shipped to the shoe factory where it need only be warmed to develop its adhesive properties before use. By such procedure the fire hazard is totally eliminated in the shoe factory as the stiffener impregnated with poly vinyl acetate is non-inflammable and none of the inflammable solvents need ever enter the factory.
- The poly vinyl acetate has a property of remaining permanently flexible to some extent so that the addition of plasticisers is unnecessary, thereby doing away with the offensive odors of these materials as well as their deleterious effect on the foot and shoe leather.
- It will be understood that such plasticisers can be added to our poly vinyl acetate solution if found desirable, but as a general rule, the disadvantage of these additional compounds outweigh the advantages in as much as the poly vinyl acetate is sufficiently flexible alone.

*Example 1*

- A felt webbing is impregnated by immersion in a 50% solution of poly vinyl acetate in alcohol and dried. The dry material possesses exceptional strength and is sufficiently flexible for use in either the box toe or the heel counter of a shoe. It is only necessary to warm this material to form it into the desired shape and upon cooling it will regain its original strength. The stiffening material thus shaped can be united with the lining and the leather of the shoe by warming to approximately 60° C. or, if it is desired, the adhesive property can be developed by exposing the material to a poly vinyl acetate solvent.
- Besides the solution of poly vinyl acetate in alcohol, the following solutions can also be used in like manner: acetone, acetic ether, benzene, butyl acetate, toluene, chlorobenzene, methyl alcohol, acetals.

*Example 2*

- A solution is prepared by dissolving 45 parts by weight of polyvinyl acetate in 55 parts of ethylacetate. A sheet of cloth is impregnated by immersion with this solution, dried and used for shoe-stiffening purposes.

The invention claimed is:

1. A shoe stiffener comprising a sheet of cloth impregnated with alcohol- and benzene-soluble poly vinyl acetate.

2. A shoe stiffener comprising a sheet of felt cloth impregnated with alcohol- and benzene-soluble poly vinyl acetate.

Signed at Munich, Germany, this 16th day of May, A. D. 1929.

WILLY O. HERRMANN.  
WOLFRAM HAEHNEL.

70

75

80

85

90

95

100

105

110

115

120

125